

# United States Patent

[19]

Lee et al.

[11]

3,730,445

[45]

May 1, 1973

[54] **METHOD OF IMPROVING THE GRINDABILITY OF ALUMINA-SILICA ORES**

[75] Inventors: **Thomas E. Lee; Frederick W. Frey**, both of Baton Rouge, La.

[73] Assignee: **Ethyl Corporation**, Richmond, Va.

[22] Filed: **Mar. 24, 1972**

[21] Appl. No.: **237,994**

**Related U.S. Application Data**

[62] Division of Ser. No. 74,169, Sept. 2, 1970.

[52] U.S. Cl.....**241/23, 241/25**

[51] Int. Cl.....**B02c 23/00**

[58] Field of Search.....**241/23, 25, 18**

2,368,194 1/1945 Brenner.....**241/23 X**  
2,899,278 8/1959 Lewis.....**241/23**

*Primary Examiner*—Granville Y. Custer, Jr.

*Attorney*—Donald L. Johnson et al.

[57]

## ABSTRACT

A method of improving the grindability or grinding characteristics of aluminous clays or alumina-silica ores containing iron species by thermally treating the clays or ores at relatively high temperature in an air or oxidative atmosphere and subsequently grinding ore to a predetermined particle size, whereby the amount of fines produced on grinding are substantially less than the amount of fines produced upon grinding a comparable non-calcined ore.

[56] **References Cited**

**10 Claims, No Drawings**

**UNITED STATES PATENTS**

2,304,440 12/1942 Brenner et al.....**241/23**

## **METHOD OF IMPROVING THE GRINDABILITY OF ALUMINA-SILICA ORES**

This is a division, of application Ser. No. 74,169, filed on Sept. 20, 1970.

## BACKGROUND OF THE INVENTION

The present invention is in the broad field of metallurgy and relates primarily to the beneficiation of aluminum clays or alumina-silica ores for subsequent use in the production of aluminum-silicon alloys.

Natural clays or ores containing aluminum-silicates or alumina-silica usually contain relatively large amounts of iron species generally in the forms of ferrous and/or ferric oxide. Such iron is a harmful impurity in the production of aluminum-silicon alloys. Unless the iron species are removed from the ore prior to carbothermic reduction for producing aluminum-silicon alloys, the resulting aluminum-silicon alloy end product will contain undesirable amounts of iron. In general, the freer an aluminum-silicon alloy is of other elements, the more useful is the alloy. Alloys containing low amounts of iron are therefore extremely desirable.

The present process is primarily adapted for removing or lowering the iron species content of alumina-silica ores prior to their carbothermic reduction into aluminum-silicon alloys. It has been discovered that calcining or thermal treatment of the raw ore or aluminum clay in an air or oxidative atmosphere promotes the agglomeration of the iron containing species and their more facile separation from the aluminous material by magnetic methods. An additional benefit of the calcination or roasting is that the grinding characteristics of the ore are modified so that less fines are produced on grinding thereby resulting in a lower loss of valuable material.

It is therefore a primary object of the present invention to provide an economical method of physically beneficiating alumina-silica ores for use in the production of aluminum-silicon alloys.

## SUMMARY OF THE INVENTION

Natural alumina-silica clays or clay minerals are heated in an oxidative atmosphere to a temperature of from about 1100° C to about 1400° C for a period of about 2 hours to about 48 hours. The calcined ore is then ground and/or crushed into fine particles of a mesh size from about -40 to +400 U. S. Sieve Series. The magnetic iron values are then separated from the non-magnetic mineral values by magnetic separation.

## DESCRIPTION OF THE PREFERRED EMBODIMENT

In the preferred embodiment of the invention a natural alumina-silica clay or clay mineral such as diaspore clay previously crushed or ground to a convenient size usually about 3 mesh, U. S. Sieve Series is heated in a kiln or other suitable container to a temperature of about 1300°-1400° C in air, oxygen or other suitable oxidative atmosphere for a period of from about 2-5 hours.

Prior to calcining, the ore particles should be of a size to permit convenient handling thereof. Although the particle size of the raw ore is not critical, an initial particle size of about one-quarter inch to about one-half inch in diameter produces favorable results. After

calcining or oxidative roasting, the ore is ground to a fine particle size of about -40 on 400 mesh, U. S. Sieve Series.

The particles of ore are then magnetically separated by any suitable means. An induced roll high intensity magnetic separator has been found to be satisfactory.

Calcination in air or an oxidative atmosphere agglomerates the iron species and improves their magnetic properties enabling the iron species to be more readily removed by magnetic separation. An air flush preheated to about 1000° C and introduced during calcination of the clay or ore at a rate of about 2-3 cubic feet per minute produces exemplary results.

15 Preheating of the air or oxidation medium permits conservation of heat energy and makes the process more economical. The quantity of air, oxygen or other suitable oxidation medium should be sufficient to accomplish the desired oxidation or agglomeration. The  
20 rate the air or oxidation medium is introduced during calcining will vary with the size and type of equipment used in the process.

25 Although the present invention is suitable for beneficiation of any alumina-silica ores, it is especially useful in the beneficiation of diaspore clay and kyanite clay, or clays containing diaspore, boehmite and/or kaolinite and iron species. Although not wishing to be bound by any particular theory, it is believed that the following occurs during calcination:



The following examples are illustrative of the invention:

### EXAMPLE A

40 A composite sample of diaspore clay containing dia-  
spore, boehmite and kaolinite as predominant minerals  
and small amounts of siderite, goethite and hematite of  
about 4/40 mesh was heated in air for two hours in a  
45 furnace at a temperature of 1380°-1410° C. The resulting  
material had visible spots and nodules of magnetic  
iron oxide. The sample was crushed in a mortar and  
pestle to 100 percent minus 40 mesh. Approximately  
50 17 percent was separated with a small hand magnet.  
The magnetic fraction was black and shiny in appear-  
ance. The non-magnetic fraction still had black  
particles in it. Conversely, no magnetic fraction could  
be separated from an original non-calcined diaspore  
clay sample with the same small hand magnet.

### EXAMPLE B

A sample of diaspore clay of 4/40 mesh was heated at 1300° C for approximately six hours. The extent of agglomeration was similar to that achieved in Example A. Results comparable to those of Example A were also obtained with a non-calcined diaspore clay sample.

### EXAMPLE C

65 Two diaspore clay samples, containing diaspore, boehmite and kaolinite as predominant minerals and small amounts of siderite, goethite and hematite, of 550

grams each were calcined in air at  $1300^{\circ}\text{C} \pm 15^{\circ}\text{C}$  in a furnace for approximately six hours. The two batches were ground together for 15 minutes in a 9-inch laboratory rod mill. A wet sieve analysis of the ground mixture is shown in Table I hereinafter.

TABLE I  
Wet Sieve Analysis

| Mesh    | Wt    | Wt %  |
|---------|-------|-------|
| +30     | 173.8 | 22.3  |
| 30/40   | 123.0 | 15.8  |
| 40/100  | 313.0 | 40.2  |
| 100/200 | 103.6 | 13.3  |
| 200/270 | 33.1  | 4.2   |
| 270/400 | 30.6  | 3.9   |
| -400    | N. A. | N. A. |

The 40/100 and 100/200 mesh fractions were passed through an induced roll high-intensity magnetic separator. The separator reaches its magnetic rating of 16,000 gauss at a field current of 2.0 amperes. No direct measurement of the field strength was possible; however, assuming linearity between field current and field strength, 70-73 percent of the iron oxides was removed at a field strength of about 11,000 gauss (at 1.4 amp.). The result of these magnetic separations are set forth in Table II hereinafter.

TABLE II.—MAGNETIC SEPARATION OF DIASPORE—CLAY AT 11,000 GAUSS

| Sample No.         | Weight percent                 |                  |                                |                  | Fraction of total |                                        |                                        |           |
|--------------------|--------------------------------|------------------|--------------------------------|------------------|-------------------|----------------------------------------|----------------------------------------|-----------|
|                    | Al <sub>2</sub> O <sub>3</sub> | SiO <sub>2</sub> | Fe <sub>2</sub> O <sub>3</sub> | TiO <sub>2</sub> | Wt.               | Percent Fe <sub>2</sub> O <sub>3</sub> | Percent Al <sub>2</sub> O <sub>3</sub> | Mesh size |
| 1—{Magnetic.....   | 50.9                           | 35.8             | 10.0                           | 3.3              | 128.0             | 70.9                                   | 38.1                                   | 40/100    |
| 1—{Non-magnetic... | 54.2                           | 39.8             | 2.7                            | 3.3              | 183.9             | 29.1                                   | 61.7                                   |           |
| 2—{Magnetic.....   | 49.6                           | 33.7             | 9.8                            | 3.3              | 54.2              | 73.0                                   | 49.8                                   | 100/200   |
| 2—{...do.....      | 54.1                           | 38.8             | 3.8                            | 3.2              | 49.2              | 26.9                                   | 40.0                                   |           |

Separation summary:

40/100:  
70.9% Fe<sub>2</sub>O<sub>3</sub> removed.  
61.7% Al<sub>2</sub>O<sub>3</sub> recovered.  
2.7% Fe<sub>2</sub>O<sub>3</sub> in concentrate.

100/200:  
73.0% Fe<sub>2</sub>O<sub>3</sub> removed.  
50.0% Al<sub>2</sub>O<sub>3</sub> recovered.  
3.8% in concentrate.

EXAMPLE D

A composite sample of diaspore ore was magnetically separated and comparable samples of the diaspore ore were calcined under varying conditions and magnetically separated using an induced roll high-intensity magnetic separator. The results of these tests are set forth in Table III.

TABLE III.—PARAMETERS OF DIASPORE CLAY FOR MAGNETIC SEPARATION

| Sample No. | Percent                                   |                                          |                                        | Calcination conditions |             |                        | Separation conditions |         |
|------------|-------------------------------------------|------------------------------------------|----------------------------------------|------------------------|-------------|------------------------|-----------------------|---------|
|            | Fe <sub>2</sub> O <sub>3</sub> in product | Al <sub>2</sub> O <sub>3</sub> recovered | Fe <sub>2</sub> O <sub>3</sub> removed | Time (hr.)             | Temp. (°C.) | Atmos.                 | Field (gauss)         | Mesh    |
| 1.....     | 3.4                                       | 82.0                                     | 60.7                                   | Non-calcined           |             |                        | 12,000                | 30/400  |
| 2.....     | 2.5                                       | 82.4                                     | 62.3                                   | 5                      | 1,300       | Air.....               | 8,030                 | 30/400  |
| 3.....     | 2.3                                       | 68.9                                     | 72.6                                   | 20                     | 1,340       | Air.....               | 8,000                 | 30/400  |
| 4.....     | 3.7                                       | 65.5                                     | 58.4                                   | 2                      | 1,300       | Air <sup>2</sup> ..... | 6,400                 | 100/200 |
| 5.....     | 2.7                                       | 51.3                                     | 78.1                                   | 16                     | 1,300       | Air.....               | 8,000                 | 30/400  |

<sup>1</sup> Percent Fe<sub>2</sub>O<sub>3</sub> in product was calculated on a calcined basis. Loss on ignition was about 14%.

<sup>2</sup> Static

From the foregoing examples, it is clearly seen that the non-calcined ore samples require a higher magnetic intensity to achieve the same amount of magnetic separation as obtained with the calcined ore samples.

The results show in all cases that the calcined ore samples effected better removal of iron than the non-calcined samples except that of sample 4 of Table III

which was calcined in static air for only two hours. It is therefore apparent that flowing air or oxidative medium is preferred.

EXAMPLE E

5 Two diaspore clay samples, containing diaspore, boehmite, and kaolinite as predominant minerals and small amounts of siderite, goethite and hematite, of 670 grams each and of a particle size of 3/40 mesh were 10 tested for their grindability or grinding characteristics. One sample was calcined at  $1300^{\circ}\text{C}$  for approximately 6 hours. Each of the samples was then separately ground dry in a laboratory rod mill for 15 minutes. Subsequently the particle size of the samples and the 15 amount of each particle were determined. The calcined sample produced about 25 percent fewer fines (-400 mesh) than the non-calcined sample. The results of these tests are set forth in Table IV hereinafter.

TABLE IV

| Grindability of 3/40 Mesh<br>Calcined and Non-calcined<br>Diaspore Clay |                                           |                                           |
|-------------------------------------------------------------------------|-------------------------------------------|-------------------------------------------|
| Sample<br>Original<br>(Non-calcined<br>Calculated                       | Percent by Weight<br>Particle Size (Mesh) | Percent by Weight<br>Particle Size (Mesh) |
|                                                                         | +40                                       | 40/400                                    |
|                                                                         | 13.3                                      | 68.5                                      |
|                                                                         |                                           | 17.9                                      |
|                                                                         | 17.4                                      | 68.7                                      |
|                                                                         |                                           | 13.6                                      |

As fines are difficult to process in beneficiation treatments of ores, and are normally considered to be a waste or lost product, calcination and/or roasting of the 45 raw ore provides an economical means of substantially reducing the fines prior to further beneficiation.

The foregoing disclosure and description of the invention is illustrative and explanatory thereof and vari-

ous changes may be made within the scope of the appended claims without departing from the spirit of the invention.

65 What is claimed is:

1. A method of improving the grindability or grinding characteristics of aluminous clays or alumina-silica ores containing iron species, wherein the clays or ores are

thermally treated in an oxidative medium and subsequently grinding the ore to a predetermined particle size, whereby the amount of fines produced on grinding are substantially less than the amount of fines produced upon grinding a comparable non-calcined ore.

2. The method of claim 1, wherein the oxidative medium is air or oxygen.

3. The method of claim 1, wherein the oxidative medium is preheated to a temperature of at least about 1000°C.

4. The method of claim 1, wherein the alumina-silica ore is a diaspore clay, kyanite clay or kyanite concentrate.

5. The method of claim 1, wherein the aluminus clay contains diaspore, boehmite and kaolinite as the predominant minerals and siderite, goethite, and hematite in substantially lesser amounts.

6. The method of claim 1, wherein the alumina-silica ore is pre-crushed or ground to a particle size of about one-quarter inch to about one-half inch in diameter prior to thermal treatment.

7. The method of claim 1, wherein the alumina-silica ore is pre-processed to about 3 mesh U. S. Sieve Series prior to thermal treatment or calcining.

8. The method of claim 1, wherein the alumina-silica ore is calcined or thermally treated at a temperature of 10 from about 1100°C to about 1400°C.

9. The method of claim 1, wherein the alumina-silica ore is calcined or thermally treated for a period of at least about two hours.

10. The method of claim 1, wherein after thermal 15 treatment, the alumina-silica ore is ground and/or crushed to a particle size of about 40 mesh U. S. Sieve Series or less.

\* \* \* \* \*

20

25

30

35

40

45

50

55

60

65